

March 22, 1960

G. O. LIENHARD

2,929,414

PAPER CONTAINING FABRIC

Filed Aug. 18, 1955

Fig. 1.



Fig. 2.



Fig. 3.



Fig. 4.



Fig. 5.



INVENTOR

Gustav O. Lienhard

BY

Charles A. Harris

ATTORNEY

1

2,929,414

**PAPER CONTAINING FABRIC**

**Gustav O. Lienhard, Metuchen, N.J., assignor to Chicopee Manufacturing Corporation, a corporation of Massachusetts**

Application August 18, 1955, Serial No. 529,191

4 Claims. (Cl. 139—420)

The present invention relates to woven fabrics suitable for upholstery, more particularly to such fabrics which are suitable for automobile and outdoor upholstery and automobile seat covers.

This invention contemplates a fabric woven from a mixture of saran filaments and paper yarns. By saran is meant a copolymer of vinylidene chloride and vinyl chloride or acrylonitrile wherein the vinyl chloride or acrylonitrile is present in a lesser amount, generally below 20 percent by weight of the copolymer. This type of material is sold for extrusion by the Dow Chemical Company. By the term filaments is meant monofilaments, multifilament strands, yarns spun from saran staple, etc. The paper yarns preferably are formed from paper strips twisted and reduced by running the strips through a reducer such as generally disclosed in Rice Patent No. 436,261. However, the paper strips may be merely crumpled and reduced rather than twisted in a regular fashion.

Paper fabrics for automobile upholstery and seat covers are well known, as are similar fabrics woven entirely of saran. Generally speaking, paper upholstery fabrics are not competitive with similar saran fabrics. While the paper fabrics are much cheaper than the saran fabrics, they also are generally weaker and wear out much more quickly. Thus, they are in a different competitive class from saran fabrics.

The present invention contemplates a modified paper fabric incorporating saran, which is much cheaper than saran fabrics due to its paper content; yet is competitive with saran fabrics in the automobile field, for instance, due to the unusual amount of strength and wear resistance contributed by the saran it contains. Other advantages of the fabric of this invention over a plain saran fabric lie in its increased resistance to damage due to cigarette burns or other damage by heat and its decreased tendency to generate static electricity due to sliding over the saran.

Apparently, a hot ash or the lighted end of a cigarette will melt a hole through an all saran seat cover, for example, very quickly; in fact, as many automobile owners know only too well, more quickly than the dropped cigarette can be recovered. In the fabric of this invention, the paper yarns which are relatively inert to heat, act both to shield the saran filaments from the direct action of heat and to "insulate" them, in a sense, from one another, thereby retarding the melting of individual filaments.

According to this invention, saran filaments are interwoven with paper yarns to form a flat fabric with the saran in the warp and the paper in the fill or vice versa, or saran may be mixed with paper in both the warp and fill or either individually. Preferably, the fabric is plain woven with the paper yarns extending in one direction and the saran filaments extending in the other. The relative proportions of paper and saran in the fabric should range between 80 percent paper and 20 percent saran and 33 percent paper and 67 percent saran. Pref-

2

erably, the fabric is plain woven fairly tightly. However, similar weaves may be employed, and for certain uses such as summer-type seat covers, the resulting weave may be fairly loose to give maximum ventilation.

5 An illustrative embodiment of a fabric according to this invention is described hereinafter in connection with the drawings wherein:

Fig. 1 is an enlarged plan view of a typical fabric according to this invention, and

10 Fig. 2 is a still further enlarged sectional view along the line 2—2 of Fig. 1, and

Fig. 3 is a similarly enlarged sectional view along the line 3—3 of Fig. 1, and

15 Fig. 4 is a greater enlargement of a portion of Fig. 2, and

Fig. 5 is a similar enlargement of a portion of Fig. 3.

Referring to the drawings, there is shown a plain woven fabric having somewhat flattened saran monofilaments 11 in the warp and similarly flattened twisted paper yarns 20 12 in the fill. This fabric is relatively tightly woven, comprising approximately 40 ends per inch of saran and about 17 picks per inch of paper. With paper yarns formed from twisted strips of 16 lb. wet strength paper approximately  $1\frac{1}{2}$  inch wide and flat saran monofilaments approximately 4500 yards per lb., the paper content is approximately 61 percent of the total with the remainder, 39 percent, saran. It will be seen that most of the coverage is provided by the flattened paper yarns 25 12 which are quite close to one another, while the flattened filaments 11 lie closely over and protect the paper yarns 12 wherever the filaments cross the yarns on one side of the fabric.

30 While the fabric is relatively flat and smooth, the paper yarns 12 are slightly crimped and the saran filaments are relatively highly crimped due mainly to the weaving operation and the fact that the yarns 12 are much bulkier than the filaments 11. The "high spots" 35 13 or tips of the crimped portions of the saran filaments 11 are exposed on both sides of the fabric whenever one

40 of the filaments passes over one of the paper yarns 12. Since the saran filaments are relatively tough and dense as compared with the bulkier paper yarns, these "high spots" 35 13 tend to take most of the wear to which the fabric is subjected thereby minimizing failure due to abrasion of the paper yarns. It will be seen that "high

45 spots" 13 or exposed portions of the saran filaments 11 are spaced from one another on the face of the fabric and more or less surrounded by the adjacent portions of the intersecting paper yarns 12. Thus, the saran is partially imbedded in the paper and the exposed portions 50 13 of the filaments are "insulated" from one another, thereby minimizing heat damage to the saran and retarding the formation of holes due to contact with the lighted ends of cigarettes, etc. Due to the relatively small proportion of saran filaments exposed on the face of the fabric as opposed to the paper, the generation of static

55 electricity due to sliding over the fabric, for example, also is minimized as mentioned hereinbefore.

60 Almost any type of paper may be employed in forming the fabric of this invention, although some type of so-called twisting tissue might best be used. Generally speaking, a wet-strength twisting tissue is preferred to minimize damage by water or other liquids. Wet-strength papers of this type conventionally are produced by mixing a wet-strength resin or a rubber or latex into the paper slurry before the paper actually is formed.

65 Having now described the invention in specific detail and exemplified the manner in which it may be carried into practice, it will be readily apparent to those skilled in the art that innumerable variations, applications, modifications, and extensions of the basic principles involved

may be made without departing from its spirit and scope. Thus, the fabrics of the present invention may be employed in a host of ways that will be readily apparent to the skilled artisan. We therefore intend to be limited only on accordance with the appended patent claims.

The claims are:

1. A wear-resistant plain woven fabric comprising somewhat flattened paper yarns in one direction of the fabric and similarly flattened relatively tough and dense saran filaments in the other direction of the fabric, the saran filaments rising at the surface of the fabric where they pass over the paper yarns on at least one side of the fabric exposing portions of the saran filaments and forming wear-resistant high spots on this side of the fabric, the exposed portions of the saran filaments being spaced from one another and partially imbedded in the surrounding paper yarns and the paper yarns being relatively closely spaced from one another, the composition of said fabric ranging between about 80 percent paper and 20 percent saran and 33 percent paper and 67 percent saran.

2. A wear-resistant plain woven fabric comprising paper yarns in the filling direction of the fabric and relatively tough and dense saran filaments in the warp direction of the fabric, the saran filaments rising at the surface of the fabric where they pass over the paper yarns on at least one side of the fabric exposing portions of the saran filaments and forming wear-resistant high spots on this side of the fabric, the exposed portions of the saran filaments being spaced from one another and partially imbedded in the surrounding paper yarns and the paper yarns being relatively closely spaced from one another, the composition of said fabric ranging between about 80 percent paper and 20 percent saran and 33 percent paper and 67 percent saran.

3. A wear-resistant woven fabric comprising paper yarns in one direction of the fabric and relatively tough

and dense saran filaments in the other direction of the fabric, the saran filaments rising at the surfaces of the fabric where they pass over the paper yarns exposing portions of the saran filaments and forming wear-resistant high spots, the exposed portions of the saran filaments being spaced from one another and partially imbedded in the surrounding paper yarns, the composition of said fabric ranging between about 80 percent paper and 20 percent saran and 33 percent paper and 67 percent saran.

4. A wear-resistant woven fabric comprising paper yarns and relatively tough and dense saran filaments intersecting one another, said yarns being bulkier than said filaments and said filaments being crimped to a greater extent than said yarns, the saran filaments rising at the surface of the fabric where they pass over the paper yarns on at least one side of the fabric exposing portions of the saran filaments and forming wear-resistant high spots on this side of the fabric, the exposed portions of the saran filaments being spaced from one another and partially imbedded in the surrounding paper yarns, the composition of said fabric ranging between about 80 percent paper and 20 percent saran and 33 percent paper and 67 percent saran.

25 References Cited in the file of this patent

UNITED STATES PATENTS

|           |              |               |
|-----------|--------------|---------------|
| 1,406,208 | Miller       | Feb. 14, 1922 |
| 2,312,089 | Gobeille     | Feb. 23, 1943 |
| 2,539,301 | Foster       | Jan. 23, 1951 |
| 2,590,995 | Merrill      | Apr. 1, 1952  |
| 2,712,834 | Black et al. | July 12, 1955 |
| 2,741,108 | Rogosin      | Apr. 10, 1956 |
| 2,812,782 | Stevens      | Nov. 12, 1957 |

35 FOREIGN PATENTS

|         |               |               |
|---------|---------------|---------------|
| 373,986 | Great Britain | Nov. 28, 1930 |
|---------|---------------|---------------|